

Jan. 21, 1947.

C. D. WEST ET AL

2,414,680

PROCESS OF CRYSTAL FORMATION

Filed July 29, 1944

FIG. 1



FIG. 2



FIG. 3



FIG. 4



INVENTORS  
Cutter D. West and  
Frederick J. Sindla  
BY  
Donald L. Brown  
Attorney

## UNITED STATES PATENT OFFICE

2,414,680

## PROCESS OF CRYSTAL FORMATION

Cutler D. West and Frederick J. Binda, Cambridge, Mass., assignors to Polaroid Corporation, Cambridge, Mass., a corporation of Delaware

Application July 29, 1944, Serial No. 547,263

18 Claims. (Cl. 23—302)

1

This invention relates to crystallography and more particularly to a new process for producing single crystals of predetermined size and orientation.

One of the objects of the invention is to provide a process for growing relatively large single crystals of uniaxial material and particularly crystals of predetermined dimensions and orientation.

Another object is to provide such crystals by a process of growth from the melt under the influence of an orienting force.

Other objects of the invention are to provide a process as outlined above wherein the orienting force is a crystal of a different material from the crystal being grown, to provide such a process wherein the orienting agent is a crystal of mica, and to provide such a process which is particularly applicable to the growth of crystals of sodium nitrate and other alkali metal compounds, such as the alkali halides, and mixed crystals of alkali metal salts.

A particular object of the invention is to provide a process for growing basal sections of uniaxial crystals, such as sodium nitrate, of large size (area) in an exceedingly short time.

Further objects and advantages will in part appear and in part be pointed out in the course of the following detailed description of one or more embodiments of the invention, which are given as non-limiting examples, in connection with the accompanying drawing, in which

Figure 1 is a diagrammatic view illustrating one embodiment of the process of the invention and comprising a vertical section through a mold utilized in said process;

Figure 2 is a diagrammatic sectional view of a crystal grown in accordance with the process illustrated in Fig. 1;

Figure 3 is a view similar to Fig. 1 illustrating another modified form of the process of the invention; and

Figure 4 is a diagrammatic sectional view illustrating still another modified form of the process of the invention.

The art of growing large single crystals is relatively old and includes work with growth from solution and growth from the melt. In general, influencing of the shape of the crystal being grown has been accomplished either by seeding a solution or melt or by careful control of the conditions of growth, notably the thermal gradients, or both. The processes of the prior art are all seriously limited from the standpoint both of the size of the finished crystal and the time

2

necessary for the process. In accordance with the present invention, it has been discovered that greatly improved results are obtained both from the standpoint of the size of the finished crystal and from the standpoint of time by growing single crystals from the melt under the influence of an orienting force comprising a totally different crystalline material and particularly under the influence of mica.

An example of a uniaxial crystalline material which is particularly adapted to production by means of the process of the present invention is sodium nitrate. Fig. 1 illustrates apparatus which has been found useful in carrying out one form of the process of the invention to produce a basal section of sodium nitrate. A container such as the hollow block 10 in Fig. 1 may comprise any suitable heat insulating material such, for example, as that sold under the trade name 15 "Marinite" and defines a cavity 12 of any desired shape. Within cavity 12 there is shown a cup 14 substantially filled with molten sodium nitrate 15. Cup 14 may comprise any of a variety of materials, but preferred results have been obtained with aluminum foil approximately 0.0015-0.003 inch in thickness. Other materials may be used provided, however, that if the material be one to which sodium nitrate will adhere strongly on solidifying, the material should either have substantially the same co-efficient of thermal expansion as solid sodium nitrate, or should be readily deformable by the sodium nitrate as the latter cools. On the other hand, other rigid materials may be used provided the adhesion thereto of the sodium nitrate is not sufficient to crack the crystal on cooling. In Fig. 1 it will be noted that an annular space 16 is provided between the outside of cup 14 and block walls 18. This arrangement is not essential, but is preferred from the standpoint of convenience of handling. Element 20 in Fig. 1 represents a cleavage section of mica preferably at least sufficiently smaller in area than cup 14 to fit easily therein.

45 In the practice of the invention with the equipment shown in Fig. 1, cup 14 may be filled with ground sodium nitrate and both the hollow block and cup then placed in a suitable oven such as an electric muffle oven until the charge is 50 completely melted. Alternatively, the sodium nitrate may be melted separately and then poured into cup 14. In either case, it is preferred to heat both the melt and hollow block 10 substantially above the melting point of sodium nitrate. For example, the interior of the oven

may be raised to a temperature of the order of 700° F. in which case the temperature within the melt will be at least of the order of 675° F. Thereafter, the hollow block may for convenience be at least temporarily removed from the oven and mica 20 floated on top of melt 15. This operation will be found relatively simple, since mica is not readily wetted by the melt and will therefore float thereon in spite of its greater density. Care should be taken, however, to avoid wetting the top of the mica by the melt, and to prevent also trapping air bubbles under the mica. It does not appear that there is any particular advantage in using freshly cleaved mica nor in taking any special precautions with respect to cleaning its surface coming in contact with melt 15. On the other hand, it does appear that preferred results are obtained when the mica is as flat as possible.

After mica 20 has been put in position, it is preferable to return the hollow block to the oven for a short heating period, for example, 15 minutes, in order to counteract the effects of the cooling while the mica was added and to establish as nearly as possible a uniform temperature throughout the melt. Thereafter the hollow block and melt may be permitted to cool and the rate of cooling may be relatively rapid, preferred results having been obtained with a cooling cycle of approximately five hours to room temperature.

Care should be taken to insure that melt 15 cool from the top in order that crystallization may be initiated at the surface of mica 20 and in order to prevent the initiation of crystallization elsewhere in the melt than at the mica surface. Such control may be obtained in a variety of ways. For example, the hollow block may be allowed to remain in an oven in order to minimize convection currents around the cups, and it is also desirable to provide the hollow block with some sort of cover adapted to shield the mica and the melt from air currents. For example, a large sheet of mica may be used as a cover as indicated by the dotted lines at 22. Satisfactory results have also been obtained by removing the hollow block from the oven, providing it with a cover 22 comprising a thin layer of heat reflecting material, such as aluminum foil of the order of 0.001 inch in thickness, and then permitting the hollow block to cool to room temperature. In general, it appears that the most satisfactory results are obtained from the standpoint of absolute uniformity in the crystal if crystallization can take place in a succession of planes substantially parallel to the lower face of mica 20. The above described heating of the hollow block is also of substantial importance in preventing heat loss from the melt except from the top.

The melting point of sodium nitrate is approximately 587° F., and in the preferred practice of the invention melt 15 will have completely solidified within approximately 15-20 minutes after the initiation of crystallization at the surface of mica 20. Thereafter, the rate of cooling is substantially less important although certain precautions should be observed. The rate should not be so rapid as to exceed the resistance of the crystal to thermal stress and produce cleavage. Moreover, sodium nitrate is relatively plastic at elevated temperatures below its melting point, and care should be taken to prevent stresses tending to deform the crystal. The above-mentioned limitations on the choice of material for cup 14 are important in this connection, although it should be noted that the importance of said

choice of material decreases inversely with the area of the crystal to be grown. In other words, when the crystal is sufficiently large in area, the relatively small outer portion which may be distorted by adhesion to the walls of the cup may readily be removed by edge grinding.

Cup 14 may be removed from the solidified crystal at any convenient time during the cooling process. It appears to make no appreciable difference in the results whether it be removed after the crystal cools to room temperature or while it is still heated to temperatures as high as of the order of 400° F. If, for example, aluminum foil is used in constructing cup 14, it will readily peel from the solidified crystal. Relatively heavy spun aluminum cups have also been used successfully, and in that case it is preferred to cut the cup away from the crystal at relatively high temperatures. Mica 20 readily separates from the solidified crystal at room temperature, although it is preferred to aid the separation with a drop of water in order to minimize the danger of stresses producing either cleavage or regions of glide twinning.

When the above steps have been carried out, the product will have the appearance indicated in Fig. 2 and will comprise two principal portions. Portion 38 will be a single crystal with its axis perpendicular to the surface which was in contact with the mica as indicated by arrow 32. Portion 33 will comprise an undergrowth of randomly oriented sodium nitrate. The relative thicknesses of portions 38 and 33 will, in general, reflect the rate of cooling during the crystallizing period.

If the thermal gradients in melt 15 are carefully controlled to produce crystallization only at the mica surface, it is possible to avoid the formation of portion 33. In general, however, a certain amount of non-oriented crystal growth will result, but this is immaterial since there is a clearly defined parting plane 34 between the two crystal portions at which they may be easily separated without damage to crystal 38. Thereafter, the latter may be readily ground and polished to any desired thickness and size.

The above-described embodiment of the invention has been successfully practiced to produce single crystals of sodium nitrate of a wide variety of shapes and sizes, including circular, triangular, and rectangular, and including sizes as large as 120 square inches and one-half inch in thickness.

The crystalline structure of mica has been the subject of considerable investigation by crystallographers and is discussed in detail in "Atomic Structure of Minerals" by W. L. Bragg, Cornell University Press, 1937, "The Structure of Crystals" by R. W. A. Wyckoff, 2nd ed., The Chemical Catalogue Company, "The Crystalline State" vol. I, by W. L. Bragg, G. Bell & Sons, Ltd., 1939, and

"Introduction to Crystal Chemistry" by R. C. Evans, Cambridge University Press, 1939. It is generally agreed that the mica crystal is built up of a number of sheets comprising hexagonal networks of linked tetrahedra. These tetrahedra are formed of a single silicon atom joined to four oxygen atoms. The three oxygen atoms forming the base of the tetrahedra are each shared by two tetrahedra. The oxygen atoms forming the vertices of the tetrahedra are not shared with other tetrahedra. Two of these sheets are placed together with the vertices of the tetrahedra pointing inwards. The vertices of one sheet are cross-linked with the vertices of the other sheet by Al atoms in muscovite or by Mg or Fe atoms in phlogopite. Hydroxyl groups are also incorpo-

rated and linked to Al, Mg or Fe alone. There is thus formed a firmly bound double sheet with the bases of the tetrahedra on each outer side. The bases of the tetrahedra are symmetrically opposed as if they were mirror images across a center plane. The hexagonal rings are likewise symmetrically opposed and two of these hexagonal rings, one in each composite sheet, thus outline a large cavity in which a large potassium atom is situated. The potassium atom may be bound to all twelve oxygens in its vicinity. The potassium atoms which join two composite sheets are at the center of each of the smallest hexagons and form, with all the other potassium atoms, a plane triangular net of potassium atoms. The triangles in this net are equilateral and have a side of 5.17 Angstroms.

The potassium atoms of the triangular net are loosely bound to the oxygen atoms comprising the bases of the linked tetrahedra and it seems that this bond depends to a certain extent upon the substitution of Al for Si in the tetrahedra. In any event the number of bonds per unit area between the oxygen atoms and the potassium atoms is considerably less than the number of bonds per unit area through any other plane of the mica. The cleavage of mica is consequently along the plane in which the potassium atoms lie.

Sodium nitrate which has the same structure as calcite is a rhombohedral crystal having triangular nets of sodium atoms lying in planes perpendicular to the *c* axis of the crystal. A plane perpendicular to the *c* axis in this crystal is known as a basal plane. Therefore, the basal plane of sodium nitrate taken at the level of the sodium atoms would constitute a triangular net of sodium atoms. This triangular net is composed of equilateral triangles. The smallest triangle of the triangular net of a sodium nitrate crystal has a side of 5.06 Angstroms.

Since the side of the potassium triangular net of the mica cleavage plane is 5.17 Angstroms in the case of muscovite and 5.32 Angstroms in the case of phlogopite, it is very close to the length of the side of the sodium triangle of the sodium net of  $\text{NaNO}_3$ . It can be seen, then, that these two triangular plane atomic networks have the same geometry. They are both built up of numerous equilateral triangles having sides of substantially the same length.

When the mica plane is cleaved, half of the potassium atoms remain with one sheet, and half go with the other sheet. In a statistical manner, there thus remains on the cleavage plane of mica only half of the potassium atoms of the potassium plane, and these are scattered at random.

The following is believed to happen when  $\text{NaNO}_3$  is crystallized on a cleavage plane of mica. Half of the potassium atoms are already missing from the cleavage plane and the sodium atoms are drawn to and occupy the places formerly occupied by the potassium atoms. The remaining potassium atoms are replaced by the sodium atoms and there is thus produced and held by the mica surface a monatomic network of sodium atoms which corresponds exactly to the monatomic network of potassium atoms in the cleavage plane prior to cleavage. This monatomic network of sodium atoms will have the same geometry and substantially the same size as the normal monatomic network in a basal plane of  $\text{NaNO}_3$  taken through the sodium level. Therefore, this monatomic network of sodium atoms will act as the foundation for the  $\text{NaNO}_3$  crystal and the  $\text{NO}_3^-$  ions will form a network layer on top of the sodium network. Next will

come another network layer of sodium atoms and then another network of  $\text{NO}_3^-$  ions, etc.

The exchange of sodium atoms for potassium atoms is believed to take place in the manner described above, since it is known that the potassium atoms are readily exchanged for other cations in solution and consequently it is believed that this exchange will take place with the sodium cation in the  $\text{NaNO}_3$  melt.

The above embodiment of the process of the invention is subject to relatively wide variation without producing appreciable changes in the product. In this connection, attention should particularly be called to the fact that the necessity of strict control of all conditions depends to a considerable extent on the quality desired in the product. In other words, if it is desired to produce a single crystal having the highest possible degree of uniformity from the standpoint of orientation and optic axis, then the greatest care should be exercised to minimize conditions tending to produce strain either during crystallization or during the cooling period, and particularly during the earlier cooling period when the crystal is more plastic. On the other hand, if perfect orientation is not essential in the product, the conditions of cooling are much less critical and, in fact, large single crystals have been successfully grown under conditions of forced cooling such that the entire time necessary to reduce the temperature of the melt and crystal to room temperature is only of the order of 15 minutes. In general it may be stated that the necessity for care in avoiding cleavage from too rapid cooling increases with the thickness of the crystal, and preferred results have been obtained by following the cooling procedure outlined above and controlling the rate to a cycle of approximately three hours from approximately 700° F. to approximately 500° F. Thereafter, the blocks may be permitted to stand at room temperature until they have completely cooled.

It is in no way essential to follow the practice above described of floating the mica on the melt and causing crystallization to proceed from the top downwards in the melt. Excellent results have been obtained either by sinking the mica to the bottom of the melt and causing crystallization to proceed in an upward direction, or by using a relatively deep cup and inserting the mica with its cleavage face perpendicular to the surface of the melt and either at the side or the middle of the cup, in which case it is preferable to keep the melt fluid and draw the mica very slowly therefrom. Apparatus for carrying out the first of these variations is illustrated in Fig. 3.

Cup 40 and hollow block 42 in Fig. 3 correspond to cup 14 and hollow block 10 in Fig. 1, but instead of positioning cup 40 within mold cavity 44, it is mounted upon a plate or block 45 of heat conducting material such, for example, as brass or aluminum. It will also be noted that mica 46 in Fig. 3 lies on the bottom of cup 40 with melt 48 filling most of the remainder of the cup.

In practicing the form of the invention illustrated in Fig. 3, mica 46 may be placed within cup 40 either before or after charge 48 is melted. For example, mica 46 may be placed in the cup and the latter then substantially filled with ground sodium nitrate. The cup and charge, preferably already mounted on plate 45, may then be placed within an oven and heated until the charge is completely melted. Thereafter hollow block 42 may be mounted over cup 40 as shown in Fig. 3 and the whole may be permitted to cool either by shutting off the heat in the oven wherein

the charge was melted, or by simply permitting the cup and plate 45 to stand at room temperature until it has cooled. The use of plate 45 as the conducting material tends to induce the flow of heat from the melt at the bottom of cup 40 and this procedure is aided by the insulating properties of hollow block 42. When the entire melt has solidified, it will have substantially the same appearance as has already been described in connection with Fig. 2. An advantage of this form of the invention moreover lies in the fact that any bubbles which may form within the melt rise to the top instead of collecting at the mica surface as is sometimes the case when the process is practiced in the manner illustrated in Fig. 1. For many purposes therefore, this form of the process gives preferred results.

The process of the present invention is not limited to sodium nitrate nor to the use of mica as the orienting force, although preferred results have been obtained with mica. Other crystals which fulfill the above conditions may be used provided that they also are not structurally altered at the fusion temperature of the new crystal and provided they may be detached therefrom without damage to the new crystal. This last essential is particularly aided by flexibility as in the case of mica. It is also preferred, but not essential, that the orienting substance and new crystal have substantially matching coefficients of thermal expansion in the plane of contact therebetween.

Among the other crystals which have been successfully grown from mica in sections perpendicular to a three-fold axis by means of the process of the invention are cubic alkali halides, such as potassium iodide, potassium bromide, rubidium iodide, sodium iodide, and mixed crystals such as mixed alkali halides and mixtures of sodium nitrate with, for example, silver nitrate. The basic requirements determining whether a new crystal may be grown by means of the process of the invention are that as the atoms are drawn to and held by the mica or other surface, the atoms will form a network which will constitute the first layer of the crystal to be formed. This monatomic network does not have to be exactly the same size as the size of the network in a plane of the final crystal, but it should be of substantially the same size.

It can be seen that a number of the alkali halides will satisfy the above-stated basic requirements. This is due to the crystalline structure of the alkali halides which are cubic. As can be seen by studying the crystalline structure of a cubic alkali halide, a plane perpendicular to one of the body diagonals will have therein a triangular network of alkali metal atoms. These triangles are equilateral triangles and the sides of the triangles have lengths quite near the lengths of the sides of the triangles in the potassium triangular net of mica cleavage plane. For instance, potassium bromide and potassium iodide have lengths of 4.81 and 5.16 Angstroms at their respective melting points. It will be understood, however, that the process essentially comprises two stages, the first of which is the formation of the crystal from the melt, and the second of which is the cooling of the new crystal to room temperature. It is possible to form new crystals by the process of the invention at the crystallizing temperature without being able to complete successfully the subsequent cooling stage. This is particularly true in the case of crystals such as potassium nitrate which have a polymorphic transition below the melting point and which

cannot be successfully cooled without transforming to a polycrystalline aggregate.

It is desirable to use a still further modification of the invention in practicing its process in connection with alkali halides, owing to the fact that the latter generally have coefficients of thermal expansion substantially different from that of the materials otherwise found most suitable for use in the cups. The preferred cup material when growing alkali halide crystals is platinum, but the adhesion thereto of the solidifying crystal melt is nevertheless so great as to tend to cause shattering of the crystal while cooling to room temperature after formation. In order to overcome this tendency, it has been found desirable to remove the mica with the crystal adhering thereto before the entire melt has solidified. A convenient way of accomplishing this step is illustrated in Fig. 4.

Mica disk 50 in Fig. 4 is illustrated as supported by three or more fine wires 52, which may comprise copper, gold or any other suitable metal capable of withstanding the temperature of the process and may be fixed in any suitable way to the edges of the mica. In carrying out this embodiment of the process of the invention, a cup 54 may be first substantially filled with the desired alkali halide melt 55, and mica 50 may then be lowered until its surface just touches the surface of the melt. This step may be more easily controlled if the cup is of at least appreciably greater diameter than the mica. The melt is then permitted to cool until a crystal of sufficient thickness has grown downward from the mica in the melt, care being taken during this phase of the process to insure cooling of the melt from the top as outlined above in connection with sodium nitrate. The time necessary for this phase of the process will usually be determined by the operator himself but will in general be of the order of 10 minutes, and the mica and attached crystal should be withdrawn from the melt before the latter has completely solidified and may then be transferred to an oven for slow cooling if desired. On the other hand, it has been found that the resistance to thermal shock of alkali halide crystals, such particularly as potassium iodide and potassium bromide, is so great that said crystals may be quenched in oil without affecting their optical properties. It should be noted, however, that in view of the substantial difference between the coefficients of thermal expansion of alkali halides and mica, it is preferred to separate the newly-formed crystal from the mica at high temperatures of the order of 500° F.

The embodiment of the invention just described has certain advantages. It is particularly useful in working with alkali halide melts since the latter wet mica readily and it will not float thereon as satisfactorily as in the case of sodium nitrate. The arrangement of wires 52, illustrated in Fig. 4, is of considerable advantage in aiding to keep the mica centered symmetrically with respect to the cup. Another advantage of this form of the invention is that choice of material for use in cup 54 becomes less important and highly satisfactory results have been obtained with materials such as porcelain, which would not otherwise lend themselves to the practice of the invention.

Since certain changes in carrying out the above process may be made without departing from its scope, it is intended that all matter contained in the above description or shown in the accom-

panying drawing shall be interpreted as illustrative and not in a limiting sense.

It is also to be understood that the following claims are intended to cover all the generic and specific features of the invention herein described, and all statements of the scope of the invention which, as a matter of language, might be said to fall therebetween.

What is claimed is:

1. In a process of producing a predeterminedly oriented section of a single crystal, the steps comprising forming a melt comprising said crystalline material, bringing into contact with said melt a cleavage surface of mica, and initiating crystallization of said melt on said cleavage surface by cooling said melt adjacent said surface at a faster rate than the remainder of said melt.

2. In a process of producing a predeterminedly oriented section of a single crystal, the steps comprising forming a melt comprising said crystalline material, bringing into contact with said melt a cleavage surface of mica, initiating crystallization of said melt on said cleavage surface by cooling said melt adjacent said surface at a faster rate than the remainder of said melt, continuing crystallization of said melt on said cleavage surface by maintaining a thermal gradient in said melt from said surface and in a direction substantially perpendicular thereto, and cooling said newly formed crystal to room temperature.

3. In a process of producing a basal section of sodium nitrate, the steps comprising forming a melt comprising sodium nitrate, bringing into contact with said melt a cleavage surface of mica, initiating crystallization of said melt on said cleavage surface by cooling said melt adjacent said surface at a faster rate than the remainder of said melt, and continuing crystallization of said melt on said cleavage surface by maintaining a thermal gradient in said melt from said surface and in a direction substantially perpendicular thereto.

4. In a process of producing a basal section of sodium nitrate, the steps comprising forming a melt comprising sodium nitrate in an open vessel comprising material having such thickness and physical characteristics as to be readily deformable by sodium nitrate cooling therein from the melt to room temperature, bringing into contact with said melt a cleavage surface of mica, initiating crystallization of said melt on said mica cleavage surface by cooling said melt adjacent said surface at a faster rate than the remainder of said melt, and continuing crystallization of said melt on said mica cleavage surface by maintaining a thermal gradient in said melt from said surface and in a direction substantially perpendicular thereto.

5. In a process of producing a basal section of sodium nitrate, the steps comprising forming a melt comprising sodium nitrate in an open vessel comprising material to which the adhesion of sodium nitrate in crystallizing from the melt is relatively low, initiating crystallization of said melt on said mica cleavage surface by cooling said melt adjacent said surface at a faster rate than the remainder of said melt, and continuing crystallization of said melt on a mica cleavage surface by maintaining a thermal gradient in said melt from said surface and in a direction substantially perpendicular thereto.

6. In a process of producing a basal section of sodium nitrate, the steps comprising forming a melt comprising sodium nitrate, floating on said melt a cleavage section of mica, and initiating

crystallization of said melt on said mica by cooling the surface of said melt at a faster rate than the remainder thereof.

7. In a process of producing a basal section of sodium nitrate, the steps comprising forming a melt comprising sodium nitrate in an open vessel, placing said vessel in a container having side and bottom walls comprising heat-insulating material, said container having the top thereof open and being heated to a temperature of the order of the melting point of sodium nitrate, floating on said melt a cleavage section of mica, providing said container with a top cover comprising material permitting the escape of heat therethrough more readily than the side and bottom walls of said container, and permitting said melt and container to cool until said melt has crystallized.

8. In a process of producing a basal section of sodium nitrate, the steps comprising forming a melt comprising sodium nitrate in an open vessel, positioning at the bottom of said melt a crystal of mica having a cleavage surface uppermost, mounting said vessel and melt on a support comprising heat-conducting material, covering said vessel and melt with a container having side and top walls comprising heat-insulating material, said container having the bottom thereof open and being heated to a temperature of the order of the melting point of sodium nitrate, and permitting said melt and container to cool until said melt has crystallized.

9. In a process of producing a predeterminedly oriented section of a single crystal, comprising an alkali metal compound, the steps comprising forming a melt comprising said crystalline material, bringing into contact with said melt a cleavage surface of mica, and initiating crystallization of said melt on said cleavage surface by cooling said melt adjacent said surface at a faster rate than the remainder of said melt.

10. In a process of producing a predetermined section of a crystal comprising an alkali halide, said crystal section being substantially perpendicular to a three-fold axis in said crystal, the steps comprising forming a melt comprising said alkali halide, suspending in contact with said melt a cleavage surface of mica, initiating crystallization of said melt on said mica cleavage surface by cooling the surface of said melt at a faster rate than the remainder thereof, and continuing crystallization of said melt on said mica cleavage surface by maintaining a thermal gradient in said melt from the top to the bottom thereof.

11. In a process of producing a predetermined section of a crystal comprising an alkali halide, said crystal section being substantially perpendicular to a three-fold axis in said crystal, the steps comprising forming a melt comprising said alkali halide, suspending in contact with said melt a cleavage surface of mica, continuing crystallization of said melt on said mica cleavage surface by maintaining a thermal gradient in said melt from the top to the bottom thereof, removing said mica and newly formed crystal from said melt before said melt has completely crystallized, separating said mica from said newly formed crystal at a temperature substantially above room temperature, and cooling said newly formed crystal to room temperature.

12. In a process of producing a basal section of sodium nitrate, the steps comprising forming a melt comprising sodium nitrate in an open vessel comprising aluminum, bringing into contact

with said melt a cleavage surface of mica, initiating crystallization of said melt on said mica cleavage surface by cooling said melt adjacent said surface at a faster rate than the remainder of said melt, and continuing crystallization of said melt on said mica cleavage surface by maintaining a thermal gradient in said melt from said surface and in a direction substantially perpendicular thereto.

13. A process of producing a single crystal, having a predeterminedly oriented axis and a relatively large cross-sectional area from a crystalline material which comprises the steps of forming a melt of said crystalline material, bringing into contact with said melt a single crystal of a material substantially infusible at the temperature of said melt, substantially insoluble in said melt, separable from a formed crystal and different than said melt, said second-named crystal having a plane surface thereof in contact with said melt and having said surface extending over at least a greater part of the cross-sectional area of the melt, said surface substantially defining the desired cross-sectional area of the said crystal to be formed, initiating crystallization of said melt on said crystal surface by cooling said melt adjacent said surface at a faster rate than the remainder of said melt, and separating said first-named crystal after formation from said second-named crystal.

14. A process of producing a single crystal, having a predeterminedly oriented axis and a relatively large cross-sectional area from a crystalline material which comprises the steps of forming a melt of said crystalline material, bringing into contact with said melt a single crystal of a material substantially infusible at the temperature of said melt, substantially insoluble in said melt, separable from a formed crystal and different than said melt, said second-named crystal having a plane surface thereof in contact with said melt and having said surface extending over at least a greater part of the cross-sectional area of the melt, said surface substantially defining the desired cross-sectional area of the said crystal to be formed, said crystal surface having an atomic structure capable of drawing out of the melt and holding a monatomic layer of atoms in a predetermined network, constituting the first layer of the crystal to be formed, said predetermined network having the same geometry as, and substantially the same size as, a like atomic network in the final formed crystal, initiating crystallization of said melt on said crystal surface by cooling said melt adjacent said surface at a faster rate than the remainder of said melt, and separating said first-named crystal after formation from said second-named crystal.

15. A process of producing a single crystal, having a predeterminedly oriented axis and a relatively large cross-sectional area from a crystalline material which comprises the steps of forming a melt of said crystalline material, placing on the surface of said melt a single crystal of a material substantially infusible at the temperature of said melt, substantially insoluble in said melt, separable from a formed crystal and different than said melt, said second-named crystal having a plane surface thereof in contact with said melt and having said surface extending over at least a greater part of the cross-sectional area of the melt, said surface substantially defining the desired cross-sectional area of the said crystal to be formed, said crystal surface having an atomic structure capable of drawing out of the

melt and holding a monatomic layer of atoms in a predetermined network constituting the first layer of the crystal to be formed, said predetermined network having the same geometry as, and substantially the same size as, a like atomic network in the final formed crystal, initiating crystallization of said melt on said crystal surface by cooling said melt adjacent said surface at a faster rate than the remainder of said melt, and separating said first-named crystal after formation from said second-named crystal.

16. A process of producing a single crystal, having a predeterminedly oriented axis and a relatively large cross-sectional area from a crystalline material which comprises the steps of forming a melt of said crystalline material, positioning at the bottom of said melt a single crystal of a material substantially infusible at the temperature of said melt, substantially insoluble in said melt, separable from a formed crystal and different than said melt, said second-named crystal having a plane surface thereof in contact with said melt and having said surface extending over at least a greater part of the cross-sectional area of the melt, said surface substantially defining the desired cross-sectional area of the said crystal to be formed, said crystal surface having an atomic structure capable of drawing out of the melt and holding a monatomic layer of atoms in a predetermined network constituting the first layer of the crystal to be formed, said predetermined network having the same geometry as, and substantially the same size as, a like atomic network in the final formed crystal, initiating crystallization of said melt on said crystal surface by cooling said melt adjacent said surface at a faster rate than the remainder of said melt, and separating said first-named crystal after formation from said second-named crystal.

17. A process of producing a single crystal, having a predeterminedly oriented axis and a relatively large cross-sectional area from a crystalline material which comprises the steps of forming a melt of said crystalline material, bringing into contact with said melt a single crystal of a material substantially infusible at the temperature of said melt, substantially insoluble in said melt, separable from a formed crystal and different than said melt, said second-named crystal having a plane surface thereof in contact with said melt and having said surface extending over at least a greater part of the cross-sectional area of the melt, said surface substantially defining the desired cross-sectional area of the said crystal to be formed, said crystal surface having an atomic structure capable of drawing out of the melt and holding a monatomic layer of atoms in a predetermined network constituting the first layer of the crystal to be formed, said predetermined network having the same geometry as, and substantially the same size as, a like atomic network in the final formed crystal, initiating crystallization of said melt on said crystal surface by cooling said melt adjacent said surface at a faster rate than the remainder of said melt, continuing crystallization of said melt on said crystal surface by maintaining a thermal gradient in said melt from said surface and in a direction substantially perpendicular thereto, and separating said first-named crystal after formation from said second-named crystal.

18. In a process of producing a basal section of sodium nitrate, the steps comprising forming a melt comprising sodium nitrate in an open vessel, placing said vessel in a container comprising heat

13

insulating walls, said walls defining an opening, said container being heated to a temperature of the order of the melting point of sodium nitrate, bringing into contact with said melt a cleavage section of mica and positioning said cleavage section adjacent said opening, providing said opening with a closure comprising material permitting

14

the escape of heat therethrough more readily than through the walls of said heat insulating container and permitting said melt and container to cool until said melt has crystallized.

CUTLER D. WEST.  
FREDERICK J. BINDA.